

## UNITED STATES PATENT OFFICE

2,321,107

## MOLD DIE METAL AND METHOD OF MAKING DIES THEREFROM

Nathan H. Schermer, Detroit, Mich., assignor of  
one-fourth to William Isler, Cleveland, OhioNo Drawing. Application April 10, 1941,  
Serial No. 387,873

13 Claims. (Cl. 148—12)

This invention relates, as indicated, to a mold die metal and method of making dies therefrom.

In the method of making mold dies, commonly known as "hobbing" or "hub-sinking," it has heretofore been customary to use for the material into which the hobb is to be sunk, a metal having low resistance to the hobb, which flows uniformly, which extrudes positively into cavities, and which generally reproduces the fine lines of the hobb.

Metals having these characteristics are difficult to find, and only one, namely Swedish iron, has been generally used, since this is the only metal which has the high ductility and low carbon content necessary for the purpose.

The disadvantages of using Swedish iron for this purpose are (1) it is relatively difficult to obtain in large quantities and is relatively expensive, and (2) it must be heat treated to produce a carburized area at the mold surface, followed by a draw to produce the desired toughness, which treatments require considerable time and involve the use of a great deal of equipment.

A primary object of the present invention is to provide a metal which has all of the aforesaid characteristics, yet is relatively inexpensive as compared with Swedish iron, and does not require a carburizing treatment or draw to produce the necessary hardness and toughness of the mold surface.

I have discovered that the metals described in my United States Patents Nos. 2,087,765 and 2,087,767, as well as those described in Bonte patent No. 2,087,764 and Forbes et al. Patents Nos. 2,087,766 and 2,087,768 are admirably adapted for use as a hobbing metal. In general, however, I have found that metals of this type described in these patents, but containing in excess of 2% carbon, are better adapted for this purpose than those containing less than 2% carbon. The analysis of such metals may be as follows:

|           | Per cent     |
|-----------|--------------|
| Carbon    | 1.00 to 4    |
| Silicon   | .45 to 1.75  |
| Manganese | Below 1.00   |
| Sulphur   | Not over .05 |
| Iron      | Balance      |

I have found, however, that a preferred analysis for hobbing metal purposes is as follows:

|            | Per cent    |
|------------|-------------|
| Carbon     | .25 to 2.50 |
| Silicon    | .80 to 1.00 |
| Manganese  | .20 to .25  |
| Sulphur    | .015 to .02 |
| Phosphorus | .015 to .02 |
| Vanadium   | .025 to .05 |
| Iron       | Balance     |

I melt the aforesaid metal and then pour it into ingots. It is desirable to retain the carbon in the combined form during solidification of the metal,

and to this end, I have found that vanadium in the amounts set forth above helps to retard primary graphitization of the metal, but does not obstruct graphitization of the metal during the final anneal to be hereinafter described. Stripping of the ingots, as soon as practicable after the metal has completely solidified helps to chill the metal and also cause the carbon to be retained in solution therein.

10 I then roll, forge or otherwise plastically deform the metal into rounds, flats, squares or other form in which hobbing metal is usually sold, and have found that such rolling, forging or other plastic deformation is best carried out at temperature 15 between about 1800° F. and about 1900° F. Due to the rather low melting point of this metal, forging at temperatures above this range may cause some difficulties, and is therefore to be avoided. Moreover, I have found it desirable to 20 give the metal a few preliminary passes or light blows to break up the dendritic or cast structure, after which the metal is again placed in the furnace to be reheated. After this preliminary treatment of the metal, further rolling or forging 25 progresses quite readily.

I then anneal or graphitize the metal, and have found that the most advantageous procedure for this purpose consists in heating the metal to about 1700° F. for about three hours, cooling the metal to about 1560° F. in about 60 minutes, cooling to about 1325° F. at the rate of 16 degrees per hour, and then cooling to 1200° F. at the rate of 10 degrees per hour. After the temperature of the metal has dropped below 1200° F., the metal 30 may be cooled to room temperature as rapidly as desired, within practical limits.

After the metal has been thus annealed or graphitized, its characteristic microstructure consists of a matrix of relatively pure ferrite, containing graphitic or temper carbon and less than .005% combined carbon. The graphitic or temper carbon has been precipitated uniformly throughout the mass. The Brinell hardness of the metal is about 92-96.

40 45 This graphitized material is well adapted as a hobbing metal, since it is quite ductile and readily lends itself to plastic deformation in the cold state. The hobbing operation, as is well known, consists in sinking a hobb into a piece 50 of hobbing metal, the hobb being a male die member, in order to form a die cavity or female die mold for the molding of plastics and the like, the hobbing metal being in the cold state during the hobbing operation. The hobbing metal which is the subject of the present invention has low resistance to the hobb, flows uniformly, extrudes positively into cavities, and generally reproduces the fine lines of the hobb.

The graphitic carbon within the metal apparently acts as a lubricant to allow inter-

granular slipping. In using my preferred analysis as a starting point in the aforesaid method of making hobbing iron, more than 2% carbon becomes available in the hobbing iron as temper or graphitic carbon.

As the mold or die has been completed, it can be heated to about 1500° F., to thereby redissolve the carbon in the iron, and then quenched directly, resulting in a hardening of the mold or die. The amount of carbon redissolved in the iron will, of course, depend upon the temperature to which the iron is heated before being quenched. I believe that at 1500° F., about 70 or 80 points of carbon are redissolved, but even this will produce a mold having quite a hard surface.

It is thus seen that I have provided a hobbing metal which has all of the advantage of Swedish iron, yet is relatively easily made in desired quantities and at relatively low cost, and the use of which obviates the prolonged carburizing treatment required in making mold dies from Swedish iron.

I claim as new and desire to secure by Letters Patent:

1. The method which comprises plastically deforming a ferrous metal containing about 1% to about 4% carbon, about .45% to about 1.75% silicon, and less than 1% manganese into a form suitable for hobbing, graphitizing the metal and then sinking a hobb in said metal.

2. The method which comprises plastically deforming a ferrous metal containing about 1% to about 4% carbon, about .45% to about 1.75% silicon, and less than 1% manganese into a form suitable for hobbing, graphitizing the metal, sinking a hobb into said metal, and then heat treating the metal to redissolve the carbon therein.

3. The method which comprises plastically deforming a ferrous metal containing about 2.25% to about 2.50% carbon, about .80% to about 1.00% silicon, and from about .025% to about .05% vanadium into a form suitable for hobbing, graphitizing the metal, sinking a hobb into said metal, and then heat treating the metal to redissolve carbon and harden.

4. The method which comprises plastically deforming a ferrous metal containing about 1% to about 4% carbon, about .45% to about 1.75% silicon, and less than 1% manganese into a form suitable for hobbing, annealing or graphitizing the metal to impart thereto a structure consisting almost entirely of a ferritic matrix having graphite or temper carbon uniformly distributed therein, sinking a hobb into said metal while in a cold state, and then reheating the metal at a temperature sufficient to cause carbon to become redissolved and the metal thereby rehardened.

5. The method which comprises plastically deforming a ferrous metal containing about 1% to about 4% carbon, about .45% to about 1.75% silicon, and less than 1% manganese into a form suitable to be hobbed, annealing the metal at a graphitizing temperature to impart thereto a structure consisting essentially of a ferritic matrix having graphite or temper carbon uniformly distributed therethrough, sinking a hobb into the graphitized metal while cold, heating the metal to about 1500° F. and quenching the metal.

6. The method which comprises plastically deforming a ferrous metal containing about 2.25% to about 2.50% carbon, about .80% to about 1.00% silicon, and about .025% to about .05% vanadium into a form suitable to be hobbed, annealing the metal at about 1700° F. for about three hours, cooling the metal to about 1560° F. in about one hour, cooling to about 1325° F. at the rate of about 16 degrees per hour, then cooling to about 1200° F. at the rate of about 10 degrees an hour, cooling to room temperature, sinking a hobb into the graphitized metal thus formed, and thereafter hardening the metal.

7. The method which comprises plastically deforming a ferrous metal containing about 2.25% to about 2.50% carbon, about .80% to about 1.00% silicon, and about .025% to about .05% vanadium at a temperature between about 1800° F. and about 1900° F. into a form suitable to be hobbed, annealing the metal at about 1700° F. for about three hours, cooling the metal to about 1560° F. in about one hour, cooling to about 1325° F. at the rate of about 16 degrees per hour, then cooling to about 1200° F. at the rate of about 10 degrees an hour, thereafter cooling to room temperature, sinking a die member into the graphitized metal thus formed to form a mold from said metal, and thereafter heat treating said mold to redissolve the carbon and harden the mold.

8. A mold formed by plastically deforming in the cold state a graphitized metal containing 1% to 4% carbon, .45 to 1.75% silicon, less than 1% manganese, and the balance substantially iron, and subsequently hardening the same.

9. A mold formed by plastically deforming in the cold state a graphitized ferrous metal containing about 2.25% to about 2.50% carbon, about .80% to about 1.00% silicon and about .025% to about .05% vanadium, and subsequently hardening the same.

10. A mold formed by sinking a hobb into a graphitized metal in the cold state containing 1% to 4% carbon, .45% to 1.75% silicon, less than 1% manganese, and the balance substantially iron, and subsequently hardening the same.

11. A mold formed by sinking a hobb into a graphitized ferrous metal in the cold state containing about 2.25% to about 2.50% carbon, about .80% to about 1.00% silicon, and about .025% to about .05% vanadium, and subsequently hardening the same.

12. The method which comprises providing in a form or shape suitable for sinking a hobb thereinto a ferrous metal containing about 1% to about 4% carbon, about .45% to about 1.75% silicon, and less than 1% manganese, graphitizing the metal, sinking a hobb in said metal, and then heat treating the metal to redissolve the carbon therein.

13. The method which comprises providing in a form or shape suitable for sinking a hobb thereinto a ferrous metal containing about 1% to about 4% carbon, about .45% to about 1.75% silicon, and less than 1% manganese, graphitizing the metal, sinking a hobb into said metal while the latter is in a cold state, and then heat treating the metal to redissolve the carbon therein.